

# UNITED STATES PATENT OFFICE.

JOSEPH F. WINNEUR, OF ROCHESTER, NEW YORK.

## LEATHER-TREATING COMPOSITION.

1,258,729.

Specification of Letters Patent. Patented Mar. 12, 1918.

No Drawing.

Application filed June 24, 1916. Serial No. 105,641.

To all whom it may concern:

Be it known that I, JOSEPH F. WINNEUR, of Rochester, in the county of Monroe and State of New York, have invented certain 5 new and useful Improvements in Leather-Treating Compositions; and I do hereby declare the following to be a full, clear, and exact description of the same.

My invention relates to leather treating 10 compositions or restorative solutions, and has for its specific object to restore the natural color and freshen the appearance of leather goods. A more particular object of my invention is to treat tan leather products 15 after they have been exposed to sunlight for a considerable time, thereby making it possible for dealers in shoes or other tan leather articles to restore their original color and make them look like new, after they have 20 been on display for a considerable time, and burned by the effects of the sun.

There is a large financial loss in the handling of leather goods generally, and particularly tan leather goods, such as shoes, 25 traveling bags and cases, due to burning or spotting of the leather or collecting of dirt thereon, that renders the goods unfit for sale, except at a sacrificial price, and it is desirable to provide a cleaning and color 30 storing solution or preparation that can be used by dealers and readily applied, and the present composition which I am about to describe in detail can be successfully used by applying it with a cloth over the surface 35 of the leather.

The essential ingredients that are employed in making the preparations are kerosene, oil of sassafras, oil of citronella and raw linseed oil, with which are preferably 40 combined certain other oils to impart a pleasant odor to the solution, although this last is not indispensable to the completed product. In the preferred embodiment of the invention, and according to which I have 45 secured quite successful results, I use the following named elements in the proportions stated, which combine to give a one-gallon solution:

|                  |                              |    |
|------------------|------------------------------|----|
| 100              | ounces water white kerosene. |    |
| $\frac{3}{4}$    | ounce oil of sassafras.      | 50 |
| 16               | ounces oil of citronella.    |    |
| $\frac{1}{4}$    | ounce oil of wintergreen.    |    |
| $\frac{1}{4}$    | ounce oil of mirbane.        |    |
| $\frac{1}{4}$    | ounce oil of birch.          |    |
| 11 $\frac{1}{2}$ | ounces raw linseed oil.      | 55 |

In the practical use of the solution, it is applied evenly over the leather and permitted to dry, after which the surface may be rubbed with a soft dry cloth to impart a greater luster to it. It is to be understood that the invention is not confined to the exact proportions or constituent parts above named, as I consider it within the province of my improvement to cover any leather 60 treating composition made from kerosene, citronella oil, sassafras oil, and raw linseed oil in any proportions found to be effective. The kerosene cleans the surface from dirt, while the citronella oil restores the leather 70 to its original color. The linseed oil has a tendency to slightly darken the leather, and the oil of sassafras fixes the color and holds it against subsequent deterioration.

I claim as my invention:

1. A leather treating composition, including as its principal constituents kerosene, oil of sassafras, oil of citronella and raw linseed oil in substantially the proportions described.

2. A leather treating composition, including kerosene, oil of sassafras, citronella oil, wintergreen oil, mirbane oil, birch oil and linseed oil in substantially the proportions described.

3. A leather treating composition, comprising four hundred parts kerosene, three parts sassafras oil, sixty-four parts citronella oil, one part wintergreen oil, one part mirbane oil, one part birch oil, and forty-six parts raw linseed oil.

JOSEPH F. WINNEUR.

Witnesses:

RUSSELL B. GRIFFITH,  
H. E. STONEBRAKER.